

March 5, 1946.

H. J. PATTISON

2,396,195

METHOD OF MAKING PATTERNS

Filed Dec. 26, 1944



Fig. 1.



Fig. 2.



Fig. 3.



Fig. 4.

INVENTOR  
Herbert J. Pattison.  
BY

Gray & Smith  
ATTORNEYS.

## UNITED STATES PATENT OFFICE

2,396,195

## METHOD OF MAKING PATTERNS

Herbert J. Pattison, Grosse Pointe Park, Mich.,  
assignor to Briggs Manufacturing Company,  
Detroit, Mich., a corporation of Michigan

Application December 26, 1944, Serial No. 569,733

12 Claims. (Cl. 22—195)

This invention relates to the production of patterns for use in preparing foundry molds utilized in the casting of metals, an object of the invention being to provide an improved method for reproducing or duplicating any existing master pattern, model or article so as to increase the productive capacity of the foundry in casting articles corresponding to the master pattern, model or article.

A further object of the invention is to provide an improved method for duplicating or reproducing a master pattern, article or model while at the same time compensating for shrinkage so that the production castings made from the pattern duplications or reproductions will in no case be undersize and in fact may, if desired, be oversize to any predetermined amount so as to allow for the removal of surface metal in finishing operations.

Another object of the invention is to provide an improved method of making patterns by reproducing an existing pattern, article or model and in such manner that the pattern reproduction will have sufficient oversize to compensate not only for shrinkage of the production casting but also for any machining operations necessary for finishing the surfaces of the casting.

Still another object of the invention is to provide a new and improved method of making patterns for use in preparing foundry molds, in which a plaster or other impression is taken of the article to be reproduced and a pattern casting is made in this impression from a metal or metallic alloy having the property of growing in size after it has congealed and stood for a period of time. When the growth of the pattern casting has proceeded to an extent giving the desired oversize, a plaster or other impression is taken of the oversize pattern after which the final pattern is cast in this impression resulting in the production of a pattern for use in preparing foundry molds having the required oversize to compensate for shrinkage of the production castings as well as any needed finishing of the surfaces thereof.

This application is a continuation in part of my application Serial No. 510,131, filed November 13, 1943.

Other objects of this invention will appear in the following description and appended claims, reference being had to the accompanying drawing forming a part of this specification wherein like reference characters designate corresponding parts in the several views.

Fig. 1 is a sectional view of a flask containing

a metal pattern or other article to be reproduced and illustrating the step of forming a plaster impression within the flask.

Fig. 2 is a sectional view of a flask containing the plaster impression and illustrating the step of forming a preliminary pattern casting within the flask.

Fig. 3 is a sectional view of a flask containing the preliminary pattern casting and illustrating the step of forming a plaster impression within the flask.

Fig. 4 is a sectional view of a flask containing the last mentioned plaster impression and illustrating the step of forming the final pattern reproduction within the flask.

Before explaining in detail the present invention it is to be understood that the invention is not limited in its application to the details of construction and arrangement of parts illustrated in the accompanying drawing, since the invention is capable of other embodiments and of being practiced or carried out in various ways. Also it is to be understood that the phraseology or terminology employed herein is for the purpose of description and not of limitation.

In the drawing there is illustrated, by way of example, a suitable master pattern, article or model 10 to be reproduced or duplicated so as to provide a pattern which may be used in preparing a foundry mold. Inasmuch as any article, such for example as a finished production casting or a master pattern or model, may be reproduced in accordance with the present invention, it will be understood that the article 10 may be of any type or category in which back-draft is eliminated so as to permit an impression to be made of the article utilizing suitable moldable material for this purpose, such as plaster or calcined gypsum. In carrying out the first step of the method the pattern or article 10 to be reproduced or duplicated, which may be of metal, wood or other suitable material, is placed within the bottom of a flask 11 supported upon a table or other suitable base. Where plaster is used to make the impression of the exposed side of the article 10, the plaster or calcined gypsum is mixed with water to produce a flowable material which is poured into the flask and allowed to set, thus providing a solid mold impression 12. The mold impression is then removed from the flask and allowed to dry.

In carrying out the second step of the invention illustrated in Fig. 2, the plaster impression 12 is reversed and placed upon a supporting plate 13 within a suitable flask 14 held

in position upon the supporting plate by means of locating dowel pins 15. Mounted upon the upper edge of the flask 14 is a cover plate or closure member 16 notched or grooved along its edges at 17 to receive the upper edges of the flask and position the cover plate 16 properly with respect thereto. This plate is provided with pairs of shrink-control depending ribs 18 extending a suitable distance within the flask and is also provided at one side thereof with an opening or hole 19 through which molten metal may be poured into the space between the cover plate and the plaster impression 12 to provide a cast impression 20 of the upper side of the plaster member 12. The ribs 18 at the underside of the cover plate 16 are bounded by a groove or channel 16a extending around the four sides of the cover plate providing in the casting 20 a continuous marginal rib 21. This marginal rib is joined by longitudinal ribs and also by a central transverse rib 22 connecting two opposite sides of the rib 21. The depending ribs 18 serve to quickly chill the metal within the cavity by rapidly conducting the heat from the molten metal away, thereby eliminating shrinkage or other defects on the working surfaces of the pattern casting. The ribs 21 and 22 provide a means by which the casting 20, when inverted, may be supported evenly upon a base in order to carry out the next step of the method.

The metal employed in forming the preliminary pattern casting 20 is preferably a low melting alloy which has very low shrinkage properties when the metal in molten state congeals or solidifies and which after solidification will grow in size when allowed to stand for a predetermined period of time. One low melting point alloy, which may be used for the purposes of the present invention, is an alloy of 58% bismuth and 42% lead known commercially as "Cerrobase" having a melting point of approximately 285° F. A casting formed from this alloy, such as the pattern casting 20, will shrink to little or no extent when the molten metal congeals and solidifies. However, after the casting has been removed from the flask and allowed to stand for a number of hours, the casting will grow in size. This growth is uniform in all directions and the amount of oversize may be predetermined by the length of time which the pattern casting 20 is allowed to stand. For example, the casting 20 after removal from the flask 14 may be permitted to grow to a predetermined amount such as .005 per inch.

When the pattern casting 20 has reached the proper oversize, it is inverted and mounted within a flask 23 and a wet plaster mix is poured into the flask to produce a mold impression 24. After the plaster material within the flask has set sufficiently it is removed therefrom and thoroughly dried. Thus, it will be seen that in the step of the method illustrated in Fig. 3 a plaster impression 24 is made of the oversize pattern casting 20 and, hence, the mold impression 24 will provide, when mounted within a flask for the purpose of casting the final pattern, an oversize cavity.

As illustrated in Fig. 4, the mold impression 24 is inverted and mounted upon a base plate 25 within a flask 26 which is anchored to the base plate by means of locating pins 27. A closure plate 28 grooved at 29 around its edges to fit over the upper edges of the flask 26 is mounted in position above the mold impression 24. As in the case of the closure plate 16, the closure mem-

ber 28 is so constructed as to control the shrinkage of the metal forming the pattern casting so that no shrinkage or defects will appear on any of the working surfaces of the final pattern to be cast in the mold impression 24. Accordingly, the member 28 is formed with a marginal groove or channel 28a extending around the four sides thereof and is also provided with cross-channels or grooves forming intervening ribs 30 of substantial depth and width. The closure or cover plate 28 is also provided with a pouring aperture 31 through which molten metal, such as brass, is poured to produce the final pattern casting 32. This casting will be provided with a continuous marginal rib 33 extending around the four sides thereof and cross-ribs 34.

Assuming that the preliminary pattern casting 20 is allowed to grow to an oversize such, for example as .005 per inch, and also assuming that the allowance necessary for the shrinkage of the metal forming the casting 32 and the shrinkage of the final production casting is in each instance .002 per inch, it will be seen that the mold impression 24 taken of the oversize pattern casting 20 will in effect have a double shrinkage value of .004 per inch plus an additional amount of oversize of .001 per inch. Having assumed, for purposes of illustration, that the metal forming the final pattern casting 32 will shrink .002 per inch, then it will be apparent that this pattern will be oversize an amount equal to .003 per inch. Thus, a production mold of plaster or other moldable material formed from the final pattern 32 will provide a casting cavity which will be oversize an amount equal to .003 per inch. This oversize will not only allow for the shrinkage of the production casting, assumed for the purposes of illustration to be at the rate of .002 per inch, but in addition will allow an amount of metal equal to .001 per inch to be removed from the surface of the production casting in finishing operations. After this amount of metal has been removed in the finishing operations the final production casting will be substantially the exact size of the master pattern, model or article 10 employed in making the initial mold impression 12.

Thus, it will be seen that by preparing the intermediate pattern casting 20 from a metal alloy having the property of growing or increasing in size after standing, it is possible to produce a final production pattern 32 having sufficient oversize to allow for shrinkage of the production casting as well as the removal of metal in any machining operations needed to finish the surfaces thereof. The allowable growth of the pattern casting 20 may be controlled within exact limits in order to meet requirements and when the predetermined oversize has been attained the plaster impression 24 is made after which the final pattern 32 is poured in the flask 26 as previously described.

The example given above is especially applicable to the production of a foundry pattern from an article, such as a production casting, which cannot be practically used as a pattern in the preparation of foundry molds since such casting has no oversize allowance for shrinkage of metal cast in such molds. In the event the article 10 is a foundry pattern, which it is desired to duplicate, and which pattern has an oversize allowance for single shrinkage, then the amount of growth of the pattern casting 20 need not be as great as would be necessary in the example given above where it is necessary to provide for double shrinkage. In such instance, assuming

the article 10 is a production pattern having a single shrinkage allowance, the pattern 20 will be allowed to grow an amount greater in size than the size of the pattern 10 sufficient to offset the shrinkage of the metal used in casting the final pattern 32 which will then be a duplication in size of the pattern 10. Additional growth to compensate for finishing operations may of course be permitted as in the example given above.

I claim:

1. The method of producing a metal pattern, including the steps of making a mold impression of an article to be reproduced, casting a pattern in said impression with a metal having the property of growing in size when allowed to stand, allowing said pattern casting to grow to a predetermined oversize, making a mold impression of said oversize pattern casting, and casting in metal a pattern from said last named mold impression.

2. The method of producing a metal pattern, including the steps of making a plaster mold impression of an article to be reproduced, casting a pattern in said impression with a metal alloy having the property of growing in size when allowed to stand, allowing said pattern casting to grow to a predetermined oversize, making a plaster mold impression of said oversize pattern casting, and casting in metal a pattern from said last named mold impression.

3. The method of producing a metal pattern, including the steps of making a mold impression of an article to be reproduced, casting a pattern in said impression with a low melting metal alloy having the property of growing in size when allowed to stand, allowing said pattern casting to grow to a predetermined oversize, making a mold impression of said oversize pattern casting, and casting in metal a pattern from said last named mold impression.

4. The method of producing a metal pattern, including the steps of forming from moldable material a mold impression of an article, casting a pattern in said impression from a metallic alloy having growth producing properties, allowing said pattern casting after cooling to stand for a predetermined period of time so as to grow uniformly to a size greater than said article, then making a mold impression from said pattern casting and casting a metal pattern in said last mold impression.

5. The method of producing a metal pattern, including the steps of forming from moldable material a mold impression of an article, casting a pattern in said impression from a metallic alloy having growth producing properties and adapted to melt at a temperature below 300° F., allowing said pattern casting after cooling to stand for a predetermined period of time so as to grow uniformly to a size greater than said article, then making a mold impression from said pattern casting and casting a metal pattern in said last mold impression.

6. The method of producing a metal pattern, including the steps of forming from moldable plaster or gypsum material a mold impression of an article, casting a pattern in said impression from a metallic alloy having growth producing properties, allowing said pattern casting after cooling to stand for a predetermined period of time so as to grow uniformly to a size greater than said article, then making a plaster mold impression from said pattern casting and casting a metal pattern in said last mold impression.

7. The method of producing a metal pattern,

including the steps of positioning an article in a flask, pouring a wet plaster mix into the flask to produce a mold impression of said article, drying and positioning said mold impression in a flask, pouring molten metal into said flask to produce a pattern casting from said mold impression, said metal having the property of growing in size when allowed to stand after a casting operation, allowing said pattern casting to stand for a predetermined period of time so as to increase a predetermined amount in size uniformly throughout all dimensions thereof, positioning the oversize pattern casting in a flask, pouring a wet plaster mix into the flask to produce a mold impression of said oversize pattern casting, drying and then positioning said last mold impression in a flask and casting a metal pattern in said last mentioned flask of said last mold impression.

8. The method of producing a metal pattern, 20 including the steps of positioning an article in a flask, pouring a wet plaster mix into the flask to produce a mold impression of said article, drying and positioning said mold impression in a flask, pouring molten metal into said flask to produce a pattern casting from said mold impression, said metal comprising a low melting alloy having the property of growing in size when allowed to stand after a casting operation, allowing said pattern casting to stand for a predetermined period of time so as to increase a predetermined amount in size uniformly throughout all dimensions thereof up to .005 per inch or less, positioning the oversize pattern casting in a flask, pouring a wet plaster mix into the flask to produce a mold impression of said oversize pattern casting, drying and then positioning said last mold impression in a flask, and casting a metal pattern in said last mentioned flask of said last mold impression.

9. The method of producing a metal pattern, 40 including the steps of making a mold impression of an article to be reproduced, casting a pattern in said impression with a metal having the property of growing or increasing uniformly in size when allowed to stand after a casting operation, 45 allowing said pattern casting to grow an oversize amount necessary to allow for double shrinkage, making a mold impression of said oversize pattern casting, and casting a pattern in said last mold impression which after shrinkage and cooling has an oversize sufficient to allow for the shrinkage of a production casting made in a mold formed from said last named pattern.

10. The method of producing a metal pattern, including the steps of making a mold impression 55 of an article to be reproduced, casting a pattern in said impression with a metal having the property of growing or increasing uniformly in size when allowed to stand after a casting operation, allowing said pattern casting to grow an oversize amount necessary to allow for the shrinkage of a metal cast in a mold prepared from said pattern casting, making a mold impression of said oversize pattern casting, and casting a metal pattern in said last mold impression.

11. The method of producing a metal pattern, including the steps of making a plaster mold impression of an article to be reproduced, casting a pattern in said impression with a low melting metal alloy having the property of growing or increasing uniformly in size when allowed to stand after a casting operation, allowing said pattern casting to grow an oversize amount necessary to allow for double shrinkage, making a plaster mold impression of said oversize pattern casting, and 70 casting a pattern in said last mold impression.

which after shrinkage and cooling has an oversize sufficient to allow for the shrinkage of a production casting made in a mold formed from said last named pattern.

12. The method of producing a metal pattern, including the steps of making a plaster mold impression of an article to be reproduced, casting a pattern in said impression with a low melting metal alloy having the property of growing or in-

creasing uniformly in size when allowed to stand after a casting operation, allowing said pattern casting to grow an oversize amount necessary to allow for the shrinkage of a metal cast in a mold prepared from said pattern casting, making a plaster mold impression of said oversize pattern casting, and casting a metal pattern in said last mold impression.

HERBERT J. PATTISON.